

July 6, 1965

R. J. HARTLE

3,193,500

EXTREME PRESSURE LUBRICANT

Original Filed Feb. 12, 1959



INVENTOR.  
ROBERT J. HARTLE

BY

*Robert J. Hartle*

ATTORNEY.

# United States Patent Office

3,193,500

Patented July 6, 1965

1

3,193,500

## EXTREME PRESSURE LUBRICANT

Robert J. Hartle, Gibsonia, Pa., assignor to Gulf Research & Development Company, Pittsburgh, Pa., a corporation of Delaware  
Original application Feb. 12, 1959, Ser. No. 792,883, now Patent No. 3,068,259, dated Dec. 11, 1962. Divided and this application June 13, 1962, Ser. No. 202,656  
8 Claims. (Cl. 252—32.7)

This application is a division of application Serial No. 792,883, filed February 12, 1959, now U.S. Patent No. 3,068,259.

This invention relates to certain compounds of molybdenum and tungsten having particular utility as additives in lubricating oils and more particularly to lubricating oil compositions containing the same.

As is well known to those skilled in the art, un compounded lubricating oils frequently fail to provide satisfactory lubrication to surfaces engaging under extreme pressure. The failure of lubricants to provide proper lubrication under high operating pressures results in the rubbing surfaces of machinery suffering considerable wear even to such an extent where they must be replaced.

This invention is based upon the discovery that certain compounds of molybdenum and tungsten which when blended in minor proportions with lubricating oils impart to the resulting composition significantly improved extreme pressure characteristics.

The compounds which have been found particularly useful as addition agents in lubricating oils according to the invention are molybdenum and tungsten salts of organic substituted dithiophosphoric acids having the general formula:



in which R is an oil-solubilizing organic radical such as aryl, alkyl, alkoxyalkyl, aralkyl, cycloalkyl, aryloxyalkyl, acylaryl and alkoxyaryl radicals; M is molybdenum or tungsten and X is a halogen or sulfur, y is the valency of the metal M, z is an integer of at least one but less than the valency of the metal M and represents the number of dithiophosphate ester groups in the product, and v is the valency of X. More specifically, R in the above general formula is selected from the group consisting of phenyl, caprolyphenyl, alkyl, cycloalkyl, alkylphenyl, alkylphenoxyl and alkoxyphenyl radicals wherein said alkyl radical contains 4 to 30 carbon atoms, said cycloalkyl radical contains 5 to 6 carbon atoms, the alkyl portion of said alkylphenyl radical contains 1 to 8 carbon atoms, the alkyl portions of said alkylphenoxyl radical contain 2 to 5 carbon atoms and the alkyl portion of said alkoxyphenyl radical contains 2 to 4 carbon atoms. More specifically, compounds of this class include a molybdenum or tungsten salt of dialkyl dithiophosphates and dicycloalkyl dithiophosphates such as dibutyl dithiophosphate, butyl hexyl dithiophosphate, amyl octyl dithiophosphate, dihexyl dithiophosphate, di-n-octyl dithiophosphate, diisooctyl dithiophosphate, didecyl dithiophosphate, dilauryl dithiophosphate, dihexadecyl dithiophosphate, dioctadecyl dithiophosphate, dicyclopentyl dithiophosphate, dicyclohexyl dithiophosphate, and so forth. Those dialkyl dithiophosphates in which the alkyl group has at least 4 carbon atoms and preferably more than 6 carbon atoms as for example from 6 to 30 are preferred since the longer alkyl chains tend to increase the solubility of the dithiophosphates in lubricating oils. The molybdenum and tungsten diaryl dithiophosphates and the diaryl dithiophosphates in which the aryl group bears an alkyl or cycloal-

2

phatic group are also useful such as for example diphenyl dithiophosphate, di-2,4-diamylphenyl dithiophosphate, di-2,4-dihexylphenyl dithiophosphate, and the various di-wax substituted diaryl dithiophosphates. The diaryloxyalkyl dithiophosphates such as di-2,4-dibutylphenoxyethyl dithiophosphate, di-2,4-diamylphenoxypropyl dithiophosphate; the diacylaryl dithiophosphates such as dicaprolylphenyl dithiophosphate, and the dialkoxyaryl dithiophosphates such as diethoxyphenyl dithiophosphate, dibutoxyphenyl dithiophosphate and the like are likewise useful. The organic substituents of the compounds are not critical and can be selected from a variety of organic radicals on the basis of their ability to impart oil-solubility to the compounds.

15 The halogen containing molybdenum and tungsten salts which are utilized in compositions of the invention are prepared by reacting the desired metal halide with an alkali metal salt of a partial ester of dithiophosphoric acid. Methods of preparing the partial esters of dithiophosphoric acids and the alkali metal salts thereof are known to the art. For example, an alkali metal salt of an ester of dithiophosphoric acid can be prepared by first reacting an appropriate alcohol or hydroxyaromatic compound with phosphorus pentasulfide and then reacting the partially esterified acid thus formed with sodium or potassium hydroxide. With regard to the proportions of reactants employed in the preparation of the compounds useful in compositions of the invention, the amounts of the alkali metal salt of the dithiophosphate ester and of the molybdenum or tungsten halide can be varied considerably; however, in all cases the mols of dithiophosphate compound employed will be less than the number required for reaction with all of the halogen atoms. The principal reaction involved in preparing the compounds useful in compositions of the invention can probably be expressed by the following illustrative equation, although it is understood that it is not desired to be bound by any theory of reaction:



45 In the above equation, R, M, y and z have the meaning indicated previously and X is a halogen.

Sulfur can be made to replace part or all of the halogen in the above reaction product simply by causing hydrogen sulfide to react therewith in the presence of a tertiary amine or other acid scavenger.

50 The synthesis of the oil-soluble molybdenum and tungsten salts useful in compositions of the invention will be better understood from the following illustrative examples.

## EXAMPLE I

To a solution of 376 grams (1 mol) of sodium diisooctyl dithiophosphate in 500 milliliters of carbon tetrachloride is added 84 grams (0.31 mol) of molybdenum pentachloride in small portions over a two hour period. 60 The temperature is maintained at approximately 55° to 60° C. during the addition. The reaction mixture is permitted to stand for a time as for example overnight, and the sodium chloride which is formed in the reaction is filtered off. The carbon tetrachloride is distilled off to leave approximately 390 grams of molybdenum tri-(diisooctyl dithiophosphate) dichloride. The product is a viscous brown liquid which turns blue on exposure to air for several hours. It is soluble in the common organic solvents.

65 70 *Analysis.*—Calculated for Mo: 7.82 percent. Found for Mo: 7.78 percent.

**3**  
**EXAMPLE II**

To a solution of 316 grams (1.0 mol) of sodium dicyclohexyl dithiophosphate in 1000 milliliters of carbon tetrachloride is added 84 grams (0.31 mol) of molybdenum pentachloride in small portions over a two hour period. The temperature is maintained at approximately 55° to 60° C. during the addition. The reaction mixture is permitted to stand for a time and the sodium chloride which is formed in the reaction is filtered off. The carbon tetrachloride is distilled off to leave molybdenum tris-(dicyclohexyl dithiophosphate) dichloride.

**EXAMPLE III**

Fifty grams (0.04 mol) of the molybdenum tris-(diisooctyl dithiophosphate) dichloride as prepared in Example I is dissolved in 100 milliliters of benzene containing approximately 0.08 mol of pyridine. Hydrogen sulfide is then bubbled slowly through the solution for about 1 hour. After standing for approximately one hour, the mixture is filtered and the solvent is removed from the filtrate under reduced pressure. Upon analysis of the final product the sulfur content was found to have increased from 13.06 percent to 16.57 percent while the chlorine content decreased from 9.70 percent to 3.58 percent. The product is a brown liquid, soluble in common organic solvents.

**EXAMPLE IV**

To a solution of 330 grams (1.0 mol) of sodium dicresyl dithiophosphate in 1000 milliliters of carbon tetrachloride is added 84 grams (0.31 mol) of molybdenum pentachloride in small portions over a two hour period. The temperature is maintained at approximately 55° to 60° C. during the addition. The reaction mixture is permitted to stand for a time, as for example overnight, and the sodium chloride which is formed in the reaction is filtered off. The carbon tetrachloride is distilled off to leave molybdenum tris-(dicresyl dithiophosphate) dichloride.

**EXAMPLE V**

To a solution of 432 grams (1.0 mol) of sodium didecyl dithiophosphate in 1000 milliliters of carbon tetrachloride is added 110 grams (0.31 mol) of tungsten pentachloride in small portions over a two hour period. The temperature is maintained at approximately 55° to 60° C. during the addition. The reaction mixture is permitted to stand for a time, as for example overnight, and the sodium chloride which is formed in the reaction is filtered off. The carbon tetrachloride is distilled off to leave tungsten tris-(didecyl dithiophosphate) dichloride.

**EXAMPLE VI**

To a solution of 528 grams (1.0 mol) of sodium dioctylphenyl dithiophosphate in 1000 milliliters of carbon tetrachloride is added 110 grams (0.31 mol) of tungsten pentachloride in small portions over a two hour period. The temperature is maintained at approximately 55° to 60° C. during the addition. The reaction mixture is permitted to stand for a time and the sodium chloride which is formed in the reaction is filtered off. The carbon tetrachloride is distilled off to leave tungsten tris-(dioctylphenyl dithiophosphate) dichloride.

**EXAMPLE VII**

To a solution of 488 grams (1.0 mol) of sodium dodecyl dithiophosphate in 1000 milliliters of carbon tetrachloride is added 202 grams (1.0 mol) of molybdenum trichloride in small portions over a two hour period. The temperature is maintained at approximately 55° to 60° C. during the addition. The reaction mixture is permitted to stand for a time and the sodium chloride which is formed in the reaction is filtered off. The carbon tetrachloride is distilled off to leave molybdenum didodecyl dithiophosphate dichloride.

**4**  
**EXAMPLE VIII**

Forty-seven grams (0.04 mol) of molybdenum tris-(dicresyl dithiophosphate) dichloride as prepared in Example IV is dissolved in 100 milliliters of benzene containing approximately 0.08 mol of pyridine. Hydrogen sulfide is bubbled through the solution until precipitation of pyridine hydrochloride is complete. After standing for approximately one hour, the mixture is filtered and the solvent is removed from the filtrate under reduced pressure to leave molybdenum tris-(dicresyl dithiophosphate) sulfide.

The molybdenum and tungsten organic substituted dithiophosphates disclosed hereinabove are particularly useful as additives to lubricating oils to improve the extreme pressure characteristics thereof. When employed for this purpose, the additives are employed in lubricating oil compositions preferably in amounts ranging from about 0.05 to about 5 percent or more by weight. The exact amount of the additives to be employed will depend to a great extent upon the purpose for which the oil is intended. For example, an oil intended for use at high temperatures and high pressures should contain more of the additive as compared to the amounts required for an oil intended for less severe usage.

The lubricating oil to which the additives are added to form a lubricating composition having improved extreme pressure characteristics can be any mineral oil of lubricating viscosity such as naphthenic base, paraffinic base and mixed base lubricating oils. Synthetic lubricating oils such as polymerized olefins, organic esters such as di-2-ethyl hexyl sebacate and di-2-ethylhexyl azelate and the like, can also be used as the base oil to form a lubricating composition in accordance with the invention. If desired, blends of oils of suitable viscosity may be employed instead of a single oil.

To prepare an improved lubricating composition in accordance with the invention the additives disclosed herein can be added to the lubricating oil base directly or in the form of a mineral oil concentrate in an amount to give the desired concentration in the final lubricating composition. Slight heating of the mixture may be advantageously employed to facilitate blending of the additives in the composition.

To demonstrate the effectiveness of the molybdenum and tungsten salts of the type described above in mineral oil compositions contemplated by this invention, several comparative tests were conducted with a mineral oil alone and with the same oil blended with a commercially available extreme pressure additive. The mineral oil employed had the following inspection:

|                         |      |
|-------------------------|------|
| Gravity, ° API          | 29.7 |
| Viscosity, S.U.V. Sec.: |      |
| 100° F.                 | 326  |
| 210° F.                 | 55.5 |
| Flash OC, ° F.          | 460  |
| Fire OC, ° F.           | 510  |

A four ball wear test was conducted as follows:

Three steel balls are securely fastened so that rotation is impossible. A fourth steel ball in a rotating spindle is placed so that it is entirely supported by the other three balls forming a pyramid. The three immobile steel balls and the rotating single steel ball are forced into contact with each other in response to a vertically applied load. Sufficient test lubricant is poured into a test cup to cover the three lower balls at a predetermined depth. The spindle is revolved at 1800 r.p.m. while electrical heating units heat the oil to a temperature of 248° F. At the conclusion of the test, wear is measured by examination of the scars on the clean surfaces of the three stationary balls; the two maximum right angle diameters of each wear scar being measured to the closest 0.01 millimeter and averaged. The antiwear properties are rated by the difference in the scar diameters.

The results of the test are given below in Table I.

Table I

| Compound added                                          | Percent concentration | Lever load (kilograms) | Average scar diameter |
|---------------------------------------------------------|-----------------------|------------------------|-----------------------|
| None (oil alone)                                        | 0                     | 10                     | 0.56                  |
| Zinc diisooctyl dithiophosphate                         | 0.5                   | 20                     | 0.72                  |
|                                                         | 0.5                   | 30                     | 1.45                  |
|                                                         | 0.5                   | 40                     | 0.40                  |
|                                                         | 0.5                   | 50                     | 0.65                  |
|                                                         | 1.0                   | 20                     | 0.89                  |
|                                                         | 1.0                   | 30                     | 0.30                  |
|                                                         | 1.0                   | 40                     | 0.35                  |
|                                                         | 1.0                   | 50                     | 0.68                  |
| Molybdenum tris-(diisooctyl-dithiophosphate) dichloride | 0.5                   | 30                     | 0.93                  |
|                                                         | 0.5                   | 40                     | 0.65                  |
|                                                         | 0.5                   | 50                     | 0.63                  |
|                                                         | 1.0                   | 30                     | 0.70                  |
|                                                         | 1.0                   | 40                     | 0.65                  |
|                                                         | 1.0                   | 50                     | 0.69                  |
|                                                         | 1.0                   | 60                     | 0.65                  |
|                                                         | 1.0                   | 70                     | 0.45                  |
| Compound prepared in Example III                        | 0.5                   | 30                     | 0.40                  |
|                                                         | 0.5                   | 40                     | 0.43                  |
|                                                         | 0.5                   | 50                     | 0.45                  |
|                                                         | 1.0                   | 30                     | 0.45                  |
|                                                         | 1.0                   | 40                     | 0.44                  |
|                                                         | 1.0                   | 50                     | 0.48                  |

The results recorded in Table I are shown graphically in the attached figure. Thus, curve A shows the results obtained with the oil alone. Curves B and C represent the results obtained with zinc diisooctyl dithiophosphate, a commercially available extreme pressure additive at concentrations of 0.5 and 1.0 percent respectively. Curves D and E represent the results obtained with the lubricating oil composition containing molybdenum tris-(diisooctyl dithiophosphate) dichloride at concentrations of 0.5 and 1.0 percent by weight respectively. Curves F and G represent the results obtained with a lubricating oil composition containing the reaction product of Example III at concentrations of 0.5 and 1.0 percent by weight respectively.

The curves shown in the figure clearly show the superiority of the lubricating compositions of this invention particularly in the upper pressure range. It will be seen also from the test results that only small amounts of the additives need be employed to obtain significant improvement in the extreme pressure characteristics of the lubricating composition.

In addition to the additives disclosed herein, there may be present in the lubricating composition of this invention other conventional additives such as pour point depressants, anti-rust agents, antioxidants, viscosity index improvers and the like.

It is apparent from the foregoing description that the invention provides novel lubricating compositions which are eminently satisfactory for use as lubricants in applications where high pressures and temperatures are encountered.

Those modifications and equivalents which fall within the spirit of the invention and the scope of the appended claims are to be considered part of the invention.

I claim:

1. A lubricating composition comprising a major proportion of a lubricating oil and a minor amount sufficient to confer improved extreme pressure characteristics to the composition of a compound having the formula:



wherein R is selected from the group consisting of phenyl, caproylphenyl, alkyl, cycloalkyl, alkylphenyl, alkylphenoxyalkyl and alkoxyphenyl radicals wherein said alkyl radical contains 4 to 30 carbon atoms, said cycloalkyl radical contains 5 to 6 carbon atoms, the alkyl portion of

said alkylphenyl radical contains 1 to 8 carbon atoms, the alkyl portions of said alkylphenoxyalkyl radical contain 2 to 5 carbon atoms and the alkyl portion of said alkoxyphenyl radical contains 2 to 4 carbon atoms; M is a metal selected from the group consisting of molybdenum and tungsten; X is an element selected from the group consisting of chlorine and sulfur; y is the valency of the metal M; z is an integer of at least one but less than the valency of the metal M; and v is the valency of X.

2. The lubricating composition of claim 1 wherein the said extreme pressure improvement additive is present in an amount from about 0.05 to about 5 percent by weight.

3. A lubricating composition comprising a major proportion of a lubricating oil and a minor amount sufficient to confer improved extreme pressure characteristics to the composition of a compound having the formula:



wherein R is selected from the group consisting of phenyl, caproylphenyl, alkyl, cycloalkyl, alkylphenyl, alkylphenoxyalkyl and alkoxyphenyl radicals wherein said alkyl radical contains 4 to 30 carbon atoms, said cycloalkyl radical contains 5 to 6 carbon atoms, the alkyl portion of said alkylphenyl radical contains 1 to 8 carbon atoms, the alkyl portions of said alkylphenoxyalkyl radical contain 2 to 5 carbon atoms and the alkyl portion of said alkoxyphenyl radical contains 2 to 4 carbon atoms; M is molybdenum; X is sulfur; y is the valency of molybdenum; z is an integer of at least one but less than the valency of molybdenum; and v is the valency of sulfur.

4. A lubricating composition comprising a major proportion of a lubricating oil and a minor amount sufficient to confer improved extreme pressure characteristics to the composition of a compound having the formula:



wherein R is selected from the group consisting of phenyl, caproylphenyl, alkyl, cycloalkyl, alkylphenyl, alkylphenoxyalkyl and alkoxyphenyl radicals wherein said alkyl radical contains 4 to 30 carbon atoms, said cycloalkyl radical contains 5 to 6 carbon atoms, the alkyl portion of said alkylphenyl radical contains 1 to 8 carbon atoms, the alkyl portions of said alkylphenoxyalkyl radical contain 2 to 5 carbon atoms and the alkyl portion of said alkoxyphenyl radical contains 2 to 4 carbon atoms; M is tungsten; X is sulfur; y is the valency of tungsten; z is an integer of at least one but less than the valency of tungsten; and v is the valency of sulfur.

5. A lubricating composition comprising a major proportion of a lubricating oil and a minor amount sufficient to confer improved extreme pressure characteristics to the composition of a compound having the formula:



wherein R is selected from the group consisting of phenyl, caproylphenyl, alkyl, cycloalkyl, alkylphenyl, alkylphenoxyalkyl and alkoxyphenyl radicals wherein said alkyl radical contains 4 to 30 carbon atoms, said cycloalkyl radical contains 5 to 6 carbon atoms, the alkyl portion of said alkylphenyl radical contains 1 to 8 carbon atoms, the alkyl portions of said alkylphenoxyalkyl radical contain 2 to 5 carbon atoms and the alkyl portion of said alkoxyphenyl radical contains 2 to 4 carbon atoms; M is molybdenum; X is chlorine; y is the valency of molybdenum; z is an integer of at least one but less than the valency of molybdenum; and v is the valency of chlorine.

6. A lubricating composition comprising a major proportion of a lubricating oil and a minor amount sufficient to confer improved extreme pressure characteristics to the composition of a compound having the formula:



wherein R is selected from the group consisting of phenyl, caproylphenyl, alkyl, cycloalkyl, alkylphenyl, alkylphenoxyalkyl and alkoxyphenyl radicals wherein said alkyl radical contains 4 to 30 carbon atoms, said cycloalkyl radical contains 5 to 6 carbon atoms, the alkyl portion of said alkylphenyl radical contains 1 to 8 carbon atoms, the alkyl portions of said alkylphenoxyalkyl radical contain 2 to 5 carbon atoms and the alkyl portion of said alkoxyphenyl radical contains 2 to 4 carbon atoms; M is tungsten; X is chlorine; y is the valency of tungsten; z is an integer of at least one but less than the valency of tungsten; and v is the valency of chlorine.

7. A lubricating composition comprising a major pro-

portion of a lubricating oil and a minor amount sufficient to confer improved extreme pressure characteristics to the composition of molybdenum tris-(diisooctyl dithiophosphate) dichloride.

5 8. A lubricating composition comprising a major proportion of a lubricating oil and a minor amount sufficient to confer improved extreme pressure characteristics to the composition of molybdenum tris-(diisooctyl dithiophosphate) sulfide.

10 References Cited by the Examiner

UNITED STATES PATENTS

|           |      |                |            |
|-----------|------|----------------|------------|
| 2,346,155 | 4/44 | Denison et al. | 252—32.7   |
| 2,480,673 | 8/49 | Reiff et al.   | 260—429 XR |
| 2,609,342 | 9/52 | White et al.   | 252—25     |
| 3,047,500 | 7/62 | Maston         | 252—46.4   |
| 3,050,538 | 8/62 | Hugel et al.   | 252—46.4   |

20 DANIEL E. WYMAN, Primary Examiner.

ALPHONSO D. SULLIVAN, Examiner.